

1

3,232,882

### LUBRICATING OIL COMPOSITIONS

Glenn Fuller and Forrest J. Watson, Berkeley, Calif., assignors to Shell Oil Company, New York, N.Y., a corporation of New York  
 No Drawing. Filed Mar. 28, 1962, Ser. No. 183,036  
 10 Claims. (Cl. 252—32.7)

This invention relates to oxidatively stabilized mineral lubricating oils and more particularly to mineral lubricating oil compositions which are stable under elevated temperatures and extreme pressure conditions.

It is known that certain sulfur-phosphorus containing compounds such as organic thiophosphate esters exhibit good extreme pressure properties. However, oils containing such additives are non-resistant to oxidation processes even under mild conditions and attempts to inhibit oxidation of such oil compositions by means of well known antioxidants such as alkyl phenols and aromatic amines have not been too successful. When such lubricating oil compositions are subjected to extreme conditions of temperature and pressure the situation becomes more aggravated.

It has now been discovered that mineral lubricating oils can be effectively stabilized over a wide temperature range and possess excellent extreme pressure and antiwear properties by incorporating in such oils minor amounts of each (0.01%—2%, preferably 0.1%—1%) of two additives which are: (A) an oil-soluble *p,p'*-methylene bis-phenol or monoether thereof represented by the formula



where the R's are  $C_4$ — $C_8$  tertiary alkyl groups preferably in the 2,6,2',6' positions and  $R_1$  is hydrogen or a  $C_1$ — $C_{10}$  alkyl, alkyloxy or a cycloalkyl radical and (B) an oil-soluble polysulfide of a phosphorus-containing compound having the general formula



wherein R is an oil-soluble hydrocarbyl group, such as an alkyl, aryl, aralkyl, alkaryl or cycloalkyl radical having at least 6 and preferably a straight-chain alkyl radical having from 10 to 18 carbon atoms, the  $R_1$ 's are the same or different groups selected from hydrogen, hydrocarbyl, or cationic group, such as metallic or non-metallic cationic group, such as mono or polyvalent metal (Ca, Ba, Cr, Mn, Fe, Cu, Ni, Cd) or amine, preferably an alkylamine,  $R_2$  is hydrogen or  $C_{1-4}$  alkyl radical, the X's are independently chalcogen atoms having an atomic number of from 8 to 16, such as oxygen or sulfur and y is an integer of from 2 to 5, preferably 2.

The oil soluble bisphenol compound represented by formula (A) include: 1,1-bis(3,5-ditert-butyl-4-hydroxyphenyl)methane; 1,1-bis(3,5-diisopropyl-4-hydroxyphenyl)methane; 1,1-bis(3,5-di-sec-butyl-4-hydroxyphenyl)methane; 1,1-bis(3-isopropyl-5-tert-butyl-4-hydroxyphenyl)methane; 1,1-bis(3,5-di(2-oxyethyl)-4-hydroxyphenyl)methane; 1,1-bis(3-sec-butyl-5(2-hexyl)-4-hydroxyphenyl)methane; 1,1-bis(3-isopropyl-5-(1,1,3,3-tetramethylbutyl)-4-hydroxyphenyl)methane; 1,1-bis(3-tertbutyl-5-methyl-2-hydroxyphenyl)methane; 1,1-bis(3-tert-butyl-5-methyl-2-hydroxyphenyl)ethane; 1,1-bis(3-tert-butyl-5-methyl-2-hydroxyphenyl)-propane; 1,1-bis(3-tert-butyl-5-methyl-2-hydroxyphenyl)isobutane; 1,1-bis(3-methyl-5-tert-butyl-6-hydroxyphenyl)methane; 3,5,3',5'-ditertbutyl-4-methoxy-4'-cresol) and mixtures thereof.

2

The compounds represented by formula (B), namely the polysulfids of certain phosphorus compounds preferably can be represented by the following formulas:



The  $R_1$ 's are as defined above in (II) or



or



or



A is an aliphatic amine, preferably a primary or secondary amine, such as  $C_8$ — $C_{10}$  primary straight-chain amines, e.g., octylamine, laurylamine, etc., or branched-chain primary aliphatic amines, e.g., t- $C_{8-24}$  alkylamine, such as



made by Rohm and Haas under the trade name "Primene," e.g. "Primene 81-R" and "Primene JM-T" or  $C_{5-18}$  secondary aliphatic amines, such as diethylamine, di-2-ethylhexylamine, didecylamine, or mixtures thereof, or (A) can be represented as (A<sub>1</sub>) in (B<sub>4</sub>) and then it is a polyvalent metal such as alkaline earth metals, e.g. Ca, Ba, Sr or other polyvalent metals such as Zn, Pb, Sn, Fe or Cd.

The polysulfides of alkylphosphono compounds, e.g. 2,3-dithia- or 2,3,4-trithia- or 2,3,4,5-tetrathiaalkyl phosphonic compounds are prepared by reacting a mercaptide having at least 6 carbon atoms with a halomethane phosphono compound such as chloromethane phosphonic acid or a dialkyl chloromethane phosphonate or their thio-derivatives in the presence of elemental sulfur and a suitable solvent, such as an aqueous alcoholic solution, at reflux temperature and under inert conditions until the reaction is completed which normally requires from 1 to about 5 days. The mercaptans include aliphatic mercaptans, such as hexyl, octyl, decyl, dodecyl, octadecyl mercaptans, cycloalkyl mercaptans, such as cyclohexyl mercaptan, dicyclohexyl mercaptan, aralkyl mercaptan, such as phenyldecyl mercaptan, benzyl mercaptan and the like. Instead of the mercaptans, the mercaptides can be used such as the alkali metal (Na or K) mercaptides of the above compounds. Suitable halomethane phosphonic compounds include chloromethane phosphonic acid, mono or dihydrocarbyl chloromethane phosphonates, e.g., mono or dibutyl chloromethane phosphonate, mono or di-2-ethylhexyl chloromethane phosphonate, mono or dilauryl chloromethane phosphonate, mono or diphenyl chloromethane phosphonate, mono or dicyclohexyl chloromethane phosphonate, mono or dibenzyl chloromethane phosphonate, di-butyl chloromethane di-thiophosphonate, diphenyl chloromethane di-thiophosphonate, alkali metal salts such as Na and K salts of chloromethane phosphonic acid, Na and K salts of monobutyl chloromethane phosphonic acid, Na and K salts of monodecyl chloromethane phosphonic acid and the like.

60

65

70

A preferred method of making the 2,3-dithia or 2,3,4-trithia or 2,3,4,5-tetrathiaalkylphosphonates is to react a mixture of a suitable mercapto compound, such as an alkali metal (Na or K)  $C_{10-18}$  alkyl mercaptide, elemental sulfur and a chloromethaneephosphonic acid, its ester or salt, e.g., an alkali metal (Na or K) salt of chloromethylphosphonic acid in an alcoholic solution under reflux conditions and under an inert atmosphere to form the alkylpolythiomethylphosphonate compound, e.g. the alkali metal salt of dithiaalkylphosphonic acid. The salt, for example, is then treated with a strong acid such as hydrochloric acid to spring the free dithiaalkylphosphonic acid, which can be converted into desired partial or full esters or polyvalent metal salts or amine salts for use as oil, fuel and grease additives as well as other uses. If the partial or full ester is the desired end product, then instead of starting with the salt of chloromethylphosphonic acid the ester can be used such as the mono or dialkyl ester of chloromethylphosphonic acid.

The following examples illustrate the preparation of additives for use in accordance with the present invention.

**EXAMPLE I.—DIBUTYL 2,3-DITHIATRI-DECYLPHOSPHONATE**

About 174 grams of n-decyl mercaptan was charged into a flask containing about 73 grams of KOH (85%) and 900 ml of ethanol. To the mixture 32 grams of elemental sulfur was added and the mixture refluxed until homogeneous at which time about 242.5 grams of dibutyl monochloromethylphosphonate was added and the mixture refluxed for about 24 hours. The reaction was cooled and the precipitant was separated by water dilution and extracted by repeated ether washing and thereafter dried over  $MgSO_4$  and the solvent was vacuum stripped. The end product dibutyl 2,3-dithiatridecylphosphonate was a straw yellow liquid readily soluble in mineral oil and exhibited good EP properties.

**EXAMPLE II.—MONOBUTYL 2,3-DITHIATRI-DECYLPHOSPHONATE**

About 206 grams of the product of Example I was charged into a flask containing aqueous solution of KOH in ethanol and the mixture was refluxed for 48 hours. The reaction product was acidified with dilute HCl and extracted with ether, washed and dried as in Example I, and the recovered product was monobutyl 2,3-dithiatridecylphosphonate, an oil-soluble product having good EP properties.

**EXAMPLE III.—2,3-DITHIATRIDECYL-PHOSPHONIC ACID**

Stoichiometric amounts of the potassium salt of decyl mercaptan, elemental sulfur and the potassium salt of monochloromethylphosphonic acid were dispersed in an aqueous solution of ethanol and the mixture was refluxed at 78° C. under a nitrogen atmosphere for about 1 day. The potassium 2,3-dithiatridecylphosphonate was then treated with strong hydrochloric acid to spring the acid product which was recovered by extraction with ether. The final product was 2,3-dithiatridecylphosphonic acid.

**EXAMPLE IV.—3-PHENYL 2,3-DITHIA-PROPYLPHOSPHONIC ACID**

The procedure of Example II is followed except that potassium salt of phenylmercaptan is used instead of potassium salt of decylmercaptan and the final product is 3-phenyl 2,3-dithiapropropylphosphonic acid.

**EXAMPLE V.—“PRIMENE JM-T” ( $t-C_{18}H_{37}NH_2$  to  $t-C_{24}H_{49}NH_2$ ) MONOBUTYL 2,3-DITHIATRIDECYLPHOSPHATE**

“Primene JM-T” salt of monobutyl 2,3-dithiatridecylphosphonate is prepared by reacting the product of Ex-

ample II with “Primene JM-T” in the amount sufficient to completely neutralize both acid groups, at about 50° C. in an alcoholic solution and thereafter recovering the amine salt from the alcoholic solution.

The following additional compounds may be prepared: 2,3-dithiaundecylphosphonic acid, 2,3,4-trithiahexadecylphosphonic acid, omega-cyclohexyl-2,3-dithiabutylphosphonic acid, omega-phenyl-2,3,4-trithiabutylphosphonic acid, dibutyl 2,3,4-trithiatrtradecylphosphonate, omega-phenyl-2,3-dithiatrdeciyl acid phosphonate, dibutyl-2,3-dithiatrdeciylthiaphosphonate, dibutyl phenyl-2,3-dithiamethylphosphonate, dithiaoctylcyclohexyl-2,3,4-trithiamethylthiophosphonate, diocetyl amine dodecylmercapto-methylphosphonate, diocetadecylamine omega-phenyl-2,3-dithiabutylphosphonate, tert-octadecylamine 2,3-dithiatrdeciylphosphonate, iron salt of 2,3-dithiatrdeciylphosphonic acid and mixtures thereof.

The particularly preferred additive mixtures illustrative of the present invention in mineral lubricating oil in concentrations indicated include:

- (A) Example I (0.015% P) and bis(3,5-ditert-butyl-4-hydroxyphenyl)methane (0.2%).
- (B) Example II (0.5% P) and bis(3,5-ditert-butyl-4-hydroxyphenyl)methane (0.5%).
- (C) Example III (0.02% P) and bis(3-isopropyl-5-tert-butyl-4-hydroxyphenyl)methane (0.3%).
- (D) Example IV (0.01% P) and bis(3,5-ditert-butyl-4-hydroxyphenyl)methane (0.2%).
- (E) Example I (0.02% P) and bis(3,5-ditert-butyl-4-hydroxyphenyl)methane (0.5%).
- (F) Example IV (0.12% P) and methyl ether of bis(3,5-ditert-butyl-4-hydroxyphenyl)methane.
- (G) Example V (0.015% P) and bis(3-methyl-5-tert-butyl-4-hydroxyphenyl)methane (0.2%).
- (H) Example I (0.015% P) and bis(3,5-isopropyl-4-hydroxyphenyl)methane (0.05%).
- (I) Example V (0.05% P) and bis(3,5-amyl-4-hydroxyphenyl)methane (0.01%).
- (J) Mixture of Examples I and V (50/50) (0.03% P) and bis(3,5-ditert-butyl-4-hydroxyphenyl)methane (0.5%).

The mineral lubricating oils may be derived from a variety of petroleum base stocks and are preferably paraffinic and/or naphthenic in character; they may also contain substantial proportions of hydrocarbons having aromatic character. The viscosity may vary within wide limits so that the oils may belong, for example, to SAE classes 5W, 10W, 20W, 20, 30, 40, 50, 60 or 70. Suitable oils may be derived from highly paraffinic crudes in which case distillation and/or dewaxing may be sufficient to provide a suitable base stock; chemical or selective solvent treatment may be used if desired, but is preferably kept to a minimum for economic reasons. Mixed-base crudes and even highly aromatic crudes which contain paraffinic hydrocarbons also provide suitable oil base stocks after refining by well-known techniques such as the separation of distillate fractions of suitable boiling range followed by solvent extraction with selective solvents, for example, furfural or phenol, to provide raffinate fractions, dewaxing, and chemical treatment, for example sulfuric acid treatment.

In addition to functioning as synergistic antioxidants, the additive mixtures of the present invention have been found to be extremely valuable in reducing wear and inhibiting corrosion.

In order to demonstrate the unexpected results which are obtained by use of the additive mixtures of the present invention, the Dornte oxidation test described in Industrial and Engineering Chemistry, August 1942, vol. 34, page 927 was used for evaluation, the conditions being 150° C. with Fe catalyst present, and the results are shown in Table I.

## 5

## Table I

Base: Mineral white oil  
Conditions: 150° C. Fe catalyst

| Additive Composition:                                                                                         | Induction period, hrs. | 5  |
|---------------------------------------------------------------------------------------------------------------|------------------------|----|
| Composition A (present invention)                                                                             | 122.5                  |    |
| Composition G (present invention)                                                                             | 174                    |    |
| Composition 1 [zinc diethyl dithiophosphate (0.015% P) + bis(3,5-ditert-butyl-4-hydroxyphenyl)methane (0.5%)] | 41.5                   | 10 |
| Composition [tricresylphosphate (0.2% P) + bis(3,5-ditert-butyl-4-hydroxyphenyl)methane (0.2%)]               | 11                     |    |
| Composition 3: bis(3,5-ditert-butyl-4-hydroxyphenyl)methane (0.5%)                                            | 15.5                   | 15 |
| Composition 4: Example I (0.015% P)                                                                           | 63                     |    |
| Composition 5: zinc diethyl dithiophosphate (0.015% P)                                                        | 5.5                    |    |

Compositions of this invention are useful for providing stability and other desired properties to petroleum products such as mineral lubricating oils which also contain small amounts (0.1% to 3%) of other agents such as the following: detergents such as metal organic sulfonates, e.g. neutral or basic Ca, Ba, or Zn petroleum sulfonates or non-ash forming detergents such as Acryloids of the 300 and 900 series, e.g. "Acryloid" 917, 966 or 315X which are copolymers of vinyl pyrrolidone and lauryl methacrylate of varying molecular weight such as of from 200,000 and 1,000,000 and described in Canadian Patent 592,974 or copolymers of vinyl pyridine and alkyl methacrylate as described in U.S. Patents 2,839,512, 2,889,282, 2,915,471 and 2,944,974; viscosity index improvers and pour point depressants such as the oil-soluble polymethacrylates available under the name "Acryloid" 150, 618, 710 and 768, described in U.S. Patent 2,710,842; condensation products of chlorinated paraffin wax and naphthalene; extreme pressure agents such as aliphatic amine salts of monochloromethanephosphonic acid or trichloromethanephosphonic acid, or the ester or amide of such acids; organic sulfides and mixtures thereof.

We claim as our invention:

1. A mineral lubricating oil composition comprising a major amount of mineral lubricating oil and minor amounts each sufficient to stabilize and impart extreme pressure properties to the mineral lubricating oil of an oil-soluble compound having the general formula



wherein the R<sub>1</sub>'s are selected independently from the group consisting of hydrogen, C<sub>1-4</sub> alkyl radical and an alkylamine and an oil-soluble alkylated methylene bisphenol.

2. The composition of claim 1 wherein the R<sub>1</sub>'s are C<sub>1-4</sub> alkyl radicals and the alkylated methylene bisphenol is bis(3,5-ditert-butyl-4-hydroxyphenyl)methane.

## 6

3. The composition of claim 1 wherein one of the R<sub>1</sub>'s is hydrogen and the other is a C<sub>1-4</sub> alkyl radical, and the alkylated methylene bisphenol is bis(3,5-ditert-butyl-4-hydroxyphenyl)methane.

4. The composition of claim 1 wherein one of the R<sub>1</sub>'s is a C<sub>1-4</sub> alkyl radical and the other is an alkylamine and the alkylated methylene bisphenol is bis(3,5-ditert-butyl-4-hydroxyphenyl)methane.

5. A mineral lubricating oil composition comprising a major amount of mineral lubricating oil and minor amounts each sufficient to impart stability and extreme pressure properties to the oil of a C<sub>10-18</sub> alkyl 2,3-dithiamethylphosphonic acid and bis(3,5-ditert-butyl-4-hydroxyphenyl)methane.

6. A mineral lubricating oil composition comprising a major amount of mineral lubricating oil and minor amounts sufficient to impart stability and extreme pressure properties to the oil of an ester of C<sub>10-18</sub> alkyl 2,3-dithiamethylphosphonic acid and an alkanol having from 1 to 4 carbon atoms and bis(3,5-ditert-butyl-4-hydroxyphenyl)methane.

7. A mineral lubricating oil composition comprising a major amount of mineral lubricating oil and minor amounts sufficient to impart stability and extreme pressure properties to the oil of an alkylamine salt of C<sub>10-18</sub> alkyl 2,3-dithiamethylphosphonic acid and bis(3,5-ditert-butyl-4-hydroxyphenyl)methane.

8. A mineral lubricating oil composition comprising a major amount of mineral lubricating oil and minor amounts each sufficient to impart stability and extreme pressure properties to the oil of 2,3-dithiatridecylphosphonic acid and bis(3,5-ditert-butyl-4-hydroxyphenyl)methane.

9. A mineral lubricating oil composition comprising a major amount of mineral lubricating oil and minor amounts each sufficient to impart stability and extreme pressure properties to the oil of 2,3-dithiatridecylphosphonic acid and an alkanol having from 1 to 4 carbon atoms and bis(3,5-ditert-butyl-4-hydroxyphenyl)methane.

10. A mineral lubricating oil composition comprising a major amount of mineral lubricating oil and minor amounts each sufficient to impart stability and extreme pressure properties to the oil of



salt of 2,3-dithiatridecylphosphonic acid and bis(3,5-ditert-butyl-4-hydroxyphenyl)methane.

## References Cited by the Examiner

## UNITED STATES PATENTS

- 2,807,653 9/1957 Filbey et al. ----- 252-52 X  
2,857,305 10/1958 Birum ----- 252-46.6 X  
3,041,279 6/1962 Calhoun et al. ----- 252-46.6 X

DANIEL E. WYMAN, Primary Examiner.